

## UNITED STATES PATENT OFFICE

2,238,882

## TEXTILE OIL

Alfred C. Goodings, Harry B. Marshall, and Herbert W. Lemon, Toronto, Ontario, Canada

No Drawing. Application December 21, 1939,  
Serial No. 310,340. In Canada February 2,  
1938

19 Claims. (Cl. 252—56)

This invention relates to improvements in textile oils. It includes oils of suitable grade and addition agents adapted to improve the composition, particularly to facilitate the removal of the oil from the textile to which it has been applied. In a preferred form of this invention, the addition agent is a diester formed by reaction of one of the hydroxyl groups of a polyhydric alcohol containing at least three hydroxyl groups such as glycerol, with a long chain fatty acid of at least 10 carbon atoms, and by reaction of a second hydroxyl group with a short chain aliphatic acid of less than 6 carbon atoms, preferably acetic acid or hydroxy acids such as lactic acid. The resulting diester alcohol is added to any base mineral oil of suitable color, stability and viscosity for use as a textile oil. 15

It is common practice to use oils on textile fibers, especially wool, to facilitate their manipulation through the various operations involved in the manufacture of cloth. One of the chief limiting factors on the use of mineral oils for this purpose is a difficulty encountered in their subsequent removal from the textile material by customary methods of washing or scouring. An object of this invention is to provide improved addition agents by which this difficulty is satisfactorily overcome and an oil composition containing high percentages of mineral oil is produced which meets all the requirements of a 30 good textile oil.

Textile oils are exposed, particularly during transportation and storage, to a wide range of atmospheric temperatures and it is also an important requirement of satisfactory textile oil compositions that no segregation of the constituents of the blend should occur such that a non-uniform composition of the oil may arise under conditions of use. Certain oil compositions, for example, otherwise satisfactory, are rendered commercially useless due to separation and segregation of one or more constituents of the blend when the oil is allowed to stand. Similarly, exposure to reduced temperatures may result in a disturbance of the homogeneity of composition of the oil which is not reversed by subsequent exposure to normal working temperatures. It is a further object of this invention to provide improved textile oil compositions of satisfactory washing or scouring properties, 50 which do not undergo segregation under conditions of use and which, even after exposure to severe winter temperatures, are readily rendered homogeneous on warming to room temperature.

It is desired by the textile industry that the oils to be applied to wool or other textile material be pale in color, particularly in the case of oils to be used on worsteds and high quality merchandise. Other requirements of a good 60

textile oil are freedom from liability to oxidize, to develop rancidity or odor, or to produce staining of the material to which it is applied. These requirements are all met by suitably refined mineral oils, particularly by the fuming acid-treated, or otherwise highly refined petroleum lubricating oils of low viscosity and light color.

Suitable mineral oils for use in the present invention are preferably of the following general characteristics, these being given for example only and without intending to preclude reasonable variation.

Table I

|                                          | General range | Preferred range |
|------------------------------------------|---------------|-----------------|
| Gravity, A. P. I.                        | 23-36         | 25-32           |
| Viscosity (Saybolt Universal at 100° F.) | 50-250        | 125-175         |
| Pour point                               | 0-50          | 25-35           |

The following example illustrates the difficulty of removing straight mineral oils for textiles by a scouring treatment.

25

## EXAMPLE I

Wool fabric was made to contain 5% of its weight of the oil to be tested and was then subjected to a standard scouring procedure which duplicates commercial practice and which was found to give strictly comparable and reproducible data on numerous different oils and oil blends. The composition of the scour liquor used in all cases was 0.4% soap and 0.1% soda-ash in water. After scouring, the residual oil in the fabric was determined by solvent extraction and was reported both as a percentage on the weight of the fabric and also as a percentage on the weight of original oil present on the cloth before scouring. The following are results for (1) an uncompounded mineral textile oil of the type used in preparing the improved textile oil compositions of the present invention and (2) olive oil, which is representative of a good textile oil:

|   | Type of oil    | Residual oil after scouring |                                   |
|---|----------------|-----------------------------|-----------------------------------|
|   |                | Percent on weight of fabric | Percent on weight of original oil |
| 1 | 100% olive oil | 2.25                        | 45.0                              |
| 2 | 100% olive oil | 0.24                        | 4.7                               |

It has now been found that by the incorporation in suitable mineral oils defined above of from about 2 to 10% of one or more of the improved addition agents of this invention, an oil is produced which can be readily scoured off from tex-

55

tile material and which meets all the requirements of a good textile oil for industrial use. In preferred compositions of this invention the quantity of the addition agent is of the order of 5 to 7% by volume of the base oil. Larger quantities of the addition agents up to about 20% or more may be used, particularly in preparing concentrates.

The addition agents suitable for use in this invention are diesters of polyhydric alcohols having at least three hydroxyl groups, preferably glycerol, in which one hydroxyl group is esterified with a long chain fatty acid of at least 10 carbon atoms which is preferably largely saturated and contains not more than two, preferably not more than one, double bond, and a second hydroxyl group is esterified with a short chain aliphatic acid of less than 6 carbon atoms, preferably less than 4 carbon atoms, such as, acetic acid or a hydroxy acid, such as lactic acid. Examples of suitable long chain fatty acids for the esterification are oleic acid and the acids of naturally occurring non-drying oils, including the vegetable fatty oils, such as coconut, and the animal oils, such as neat's-foot and lard oils, as well as mixtures of such acids, particularly the mixed acids obtained on hydrolysis of such naturally occurring ring oils. Erythritol and mannitol, which possess 4 and 6 hydroxy groups respectively, when partially esterified with a long chain fatty acid and a short chain aliphatic acid in the manner described above so as to leave at least one hydroxyl group unesterified, also provide compounds of value for use in this invention. The preparation of suitable diesters for use in this invention is illustrated by the following example:

#### EXAMPLE II

Coconut monoglyceride is prepared by reacting coconut oil with glycerol using preferably an excess of glycerol above that required for theoretical conversion of the coconut oil to fatty acid monoglycerides. This reaction is accomplished for example by heating 100 volumes of coconut oil with 21 volumes of glycerol at about 220° C. for five hours, using small amounts of alkali as a catalyst. This esterification reaction does not proceed entirely to completion but reaches an equilibrium in which there are small percentages of the original reactants, namely, glycerol and coconut triglyceride. If this mixture is acetylated, the free glycerol is converted to the mono- and diacetylated glycerols, which are high boiling liquids, soluble in water, insoluble in petroleum oils. The presence of these compounds in the desired coconut-acetic diglyceride is objectionable because of their insolubility in mineral oil which prevents the preparation of a completely clear textile oil solution. This difficulty can be overcome in any one of three ways

(a) The glycerol may be extracted from the coconut monoglyceride with water.

(b) The acetylated glycerol may be extracted from the coconut acetic diglyceride with water.

In either case, residual water is then removed from the extracted coconut acid ester by any suitable method as by passing a dry gas through the hot liquid with suitable agitation.

(c) Other agents which prevent separation of the acetylated glyceride from the textile oil composition, such as, liquid diglycerides of long chain fatty acids of at least 12 carbon atoms, may be added. This will be described below.

The coconut acid monoglyceride prepared as

described above, with or without prior separation of unreacted glycerine, is then acetylated by reaction with acetic anhydride. This is accomplished by heating the coconut acid monoglyceride product with 35 volumes of acetic anhydride thereby providing a slight excess of the acetylating agent. There is thus obtained a glycerol diester of the coconut acids and acetic acid which is identified for the purpose of this invention as coconut-acetic diglyceride.

Similar glycerol diesters may be prepared from neat's-foot oil and from oleic acid. Lactic acid anhydride may be used in place of the acetic anhydride to prepare corresponding diesters of a long chain fatty acid and of lactic acid. Examples of suitable glycerol diesters for use in this invention are:

20      Coconut-acetic diester of glycerol  
Neat's-foot-acetic diester of glycerol  
Neat's-foot-lactic diester of glycerol

The following scouring test data illustrate the 25 efficiency of these compounds as addition agents to mineral oils to improve ease of scouring. The compositions tested were prepared by dissolving in a mineral textile oil of the type described above, glycerol diesters in the amounts indicated in the table. The scouring test was the same as that 30 described above in Example I.

#### Mineral oil/coconut-acetic diglyceride mixtures

|    | Composition of oil                              | Residual oil                |                                   |
|----|-------------------------------------------------|-----------------------------|-----------------------------------|
|    |                                                 | Percent on weight of fabric | Percent on weight of original oil |
| 40 | 100% mineral oil                                | 2.25                        | 45.0                              |
|    | 99% mineral oil + 1% coconut-acetic diglyceride |                             |                                   |
| 45 | 98% mineral oil + 2% coconut-acetic diglyceride | 0.67                        | 13.3                              |
|    | 97% mineral oil + 3% coconut-acetic diglyceride | 0.55                        | 11.0                              |
|    | 96% mineral oil + 4% coconut-acetic diglyceride | 0.45                        | 9.0                               |
|    | 95% mineral oil + 5% coconut-acetic diglyceride | 0.33                        | 6.6                               |
| 50 | 94% mineral oil + 6% coconut-acetic diglyceride | 0.27                        | 5.4                               |
|    | 93% mineral oil + 7% coconut-acetic diglyceride | 0.21                        | 4.2                               |

#### Mineral oil/neat's-foot lactic diglyceride mixtures

|    | Composition of oil                                  | Residual oil                |                                   |
|----|-----------------------------------------------------|-----------------------------|-----------------------------------|
|    |                                                     | Percent on weight of fabric | Percent on weight of original oil |
| 60 | 100% mineral oil                                    | 2.25                        | 45.0                              |
|    | 99% mineral oil + 1% neat's-foot-lactic diglyceride | 1.90                        | 38.0                              |
| 65 | 98% mineral oil + 2% neat's-foot-lactic diglyceride | 0.85                        | 17.0                              |
|    | 97% mineral oil + 3% neat's-foot-lactic diglyceride | 0.57                        | 11.4                              |
|    | 96% mineral oil + 4% neat's-foot-lactic diglyceride | 0.52                        | 10.4                              |
|    | 95% mineral oil + 5% neat's-foot-lactic diglyceride | 0.45                        | 9.0                               |
| 70 | 94% mineral oil + 6% neat's-foot-lactic diglyceride | 0.43                        | 8.6                               |
|    | 93% mineral oil + 7% neat's-foot-lactic diglyceride | 0.43                        | 8.5                               |

Similarly, a textile oil composition containing 94% mineral oil and 6% neat's-foot-acetic digly-

eride gave a residual oil content of 0.33% on the weight of the fabric in the same scouring test.

The usual textile practice requires textile oils which can be removed from oiled textile material by ordinary methods of scouring such that not more than 0.5% of oil on the weight of material is left in the goods after a commercial scour. Suitable concentrations for the preferred textile oil compositions of this invention are thus apparent from the compositions shown to meet 10 this test in the above tables of scouring test data.

The textile oil compositions described above also undergo no segregation of any of the constituents leading to loss in scouring efficiency under any conditions of atmospheric temperatures ordinarily encountered, even including the extremely low temperatures of northern winters.

If an oil is subjected to progressively decreasing temperature, it passes from a liquid to a 20 gelatinous state. In the case of a mineral textile oil to which compounds have been added to increase the ease of scouring these addition agents may, on cooling the oil blend, precipitate out from the mineral oil while the latter is still liquid. For the oil composition to be satisfactory for textile use, it is imperative that said solidification of any of the constituents brought about by reduction of temperature should not be accompanied by a segregation leading to such non-uniform composition that portions of the oil have not the necessary good scouring properties. The fact that one constituent may solidify before another with reduction in temperature is not in itself important provided uniformity of distribution throughout the mass is not disturbed. It is further necessary that irrespective of the previous temperature conditions within the limits of atmospheric range to which the oil has been subjected, a homogeneous liquid product results when the oil is later exposed to a temperature of 50° F. The improved textile oil compositions of the present invention satisfy these requirements.

The diesters of long chain and short chain acids described above may also be used in textile oil compositions with other scouring aids such as the normally liquid mono- and di-glycerides of long chain fatty acids having at least 12 carbon atoms in the acid radical. Even though some of these normally liquid diesters tend to separate from solutions in textile mineral oils, it has been found that they may be used with the diesters of long chain and short chain acids described above and that their tendency to precipitation and segregation is thereby overcome. For example, a normally liquid diglyceride of neat's-foot oil acids which would itself partly settle out from solution in a textile mineral oil on cooling, will if mixed with neat's-foot-lactic diglyceride in suitable proportions provide a mixture of diglycerides which overcomes these difficulties of separation and which is satisfactory for use as an addition agent in the production of textile mineral oil compositions in accordance with the present invention. Examples of suitable mixtures of these diglycerides are:

Neat's-foot diglyceride and neat's-foot-lactic diglyceride

Neat's-foot diglyceride and coconut-lactic diglyceride

The effect of the addition of neat's-foot-lactic diglyceride on the precipitation of neat's-foot

diglyceride at low temperatures (5° C.) from solution in a textile mineral oil is indicated in the following table:

#### Composition of mixture in mineral oil

| % neat's foot / % neat's-foot-diglyceride | Volume of precipitation* |
|-------------------------------------------|--------------------------|
| 5/0                                       | 10                       |
| 5/1                                       | 6                        |
| 5/2                                       | 3                        |
| 5/3                                       | Negligible               |
| 5/4                                       | Negligible               |
| 5/5                                       | Negligible               |
| 0/5                                       | Negligible               |
| 4/1                                       | 4                        |
| 4/2                                       | Negligible               |
| 4/3                                       | Negligible               |
| 4/4                                       | Negligible               |

\* The volume of precipitation is expressed in arbitrary units with the figure 10 denoting the amount of precipitation taking place in a 5% solution of neat's-foot diglyceride in mineral oil (5° C.) without the addition of any neat's-foot-lactic diglyceride.

#### EXAMPLE III

The following table gives scouring test data which illustrate the effectiveness on ease of 30 scouring of additions of mixtures of neat's-foot diglyceride and neat's-foot-lactic diglyceride to a mineral textile oil of the type described above.

[A = equal parts of neat's-foot-diglyceride and neat's-foot-lactic diglyceride]

| Composition of oil     | Residual oil                |                                   |
|------------------------|-----------------------------|-----------------------------------|
|                        | Percent on weight of fabric | Percent on weight of original oil |
| 100% mineral oil       | 2.25                        | 45.0                              |
| 99% mineral oil + 1% A | 1.37                        | 27.3                              |
| 98% mineral oil + 2% A | 0.72                        | 14.3                              |
| 97% mineral oil + 3% A | 0.49                        | 9.8                               |
| 96% mineral oil + 4% A | 0.41                        | 8.2                               |
| 95% mineral oil + 5% A | 0.37                        | 7.4                               |
| 94% mineral oil + 6% A | 0.37                        | 7.4                               |
| 93% mineral oil + 7% A | 0.33                        | 6.5                               |

50 The mono- and diglycerides of the mixed fatty acids from many naturally occurring non-drying fatty oils such as neat's-foot oil and lard oil are partly solid and partly liquid at temperatures from 50 to 70° F. By cold pressing, decantation, 55 centrifuging, or other means of separating the liquid and solid portions, liquid fractions (liquid at 50° F.) of the mono- and diglycerides are obtained. These liquid monoglycerides and diglycerides are preferred for use in compositions with the glycerol diesters of long chain and short chain acids described above. The solid fractions of the mono- and diglycerides of oils such as coconut oil and neat's-foot oil are not suitable for use in these compositions. These normally solid mono- and diesters can, however, be used as illustrated 60 in Example II to prepare the mixed esters of long chain and short chain acids. For example, the normally solid fraction of the diglyceride made from neat's-foot oil can be employed in the manufacture of neat's-foot-lactic diglyceride thereby providing use for the entire neat's-foot oil and permitting marked savings in the total cost of production of the addition agents. An ex-

ample of a suitable addition agent consisting of such a mixture of diglycerides is

1 part neat's-foot diglyceride  
1 part neat's-foot-lactic diglyceride

prepared by taking the more liquid fraction of a preparation of neat's-foot diglyceride and adding to it the required proportion of neat's-foot-lactic diglyceride which has in turn been prepared from the normally solid fraction of the original neat's-foot diglyceride.

A suitable composition of the final oil mixture is

|                                      | Per cent |
|--------------------------------------|----------|
| Mineral oil.....                     | 94       |
| Neat's-foot-diglyceride .....        | 3        |
| Neat's-foot-lactic diglyceride ..... | 3        |

The liquid mono- or diglyceride may also be used in conjunction with mixed diglycerides derived from a different oil, as in the following illustrative composition:

|                                                 | Per cent |
|-------------------------------------------------|----------|
| Mineral oil.....                                | 94       |
| Coconut-acetic diester of glycerol.....         | 4        |
| Neat's-foot diglyceride (liquid fraction) ..... | 2        |

The addition of the normally liquid diglycerides to the glycerol diesters of long chain and short chain fatty acids is also of advantage in that it overcomes the insolubility in petroleum oils of any acetylated glycerols which may be left in such mixed glycerol diesters. For example, a 5% solution in a textile mineral oil of coconut-acetic diglyceride containing acetylated glycerols which are insoluble in such oil, can be completely clarified by the addition of 3% of normally liquid neat's-foot diglycerides.

The textile oil compositions described herein may be applied to the textile material in the usual manner as by spraying or sprinkling, either directly or after emulsification with water. In the case of oil emulsions, the oil is ordinarily used in about two to eight times its volume of water, with or without addition of alkali to the water. To simplify preparation of such an emulsion, it is an advantage if the oil will readily mix with water without recourse to the use of additional compounds on the part of the textile mill operative. The addition agents discussed herein are designed primarily to improve the ease of scouring of the textile oils, whether emulsified or not, and also have the effect of improving the emulsifiability of the textile oil compositions to some extent. Where it is required that the textile oil compositions should emulsify very readily in water, it is desirable to incorporate secondary addition agents into the oil for this purpose. Examples of suitable emulsifiers are the oil-soluble sulfonates, ethanolamines and the like. For example, about 3% of the mineral oil in any of the textile oil compositions described above may be replaced by an equal volume of triethanolamine. Fat solvents such as cyclohexanol (hexalin) may also be added to assist in keeping any normally solid diesters in solution.

Although emphasis has been laid on the use of mineral oils, it will be understood that the invention is applicable also to oils of animal and vegetable origin, for example, olive oil and lard oil. The addition of the diesters of glycerine, described herein, for example, to such oils, facilitates their removal from textile material, by scouring, though not to so great a degree as in the case of mineral oils.

The foregoing description is for the purpose of illustration only and various changes and alternative compositions may be made without departing from the spirit of this invention, it being intended to claim all novelty inherent in this invention as broadly as the prior art permits.

We claim:

1. A textile oil comprising a base oil having a Saybolt Universal viscosity between about 50 and 250 seconds at 100° F., and containing as a scouring assistant an effective amount of a mixed diester of a polyhydric alcohol of at least three hydroxy groups with a long chain fatty acid of at least 10 carbon atoms and not more than two double bonds and a short chain aliphatic acid of less than about 6 carbon atoms.

2. Composition according to claim 1 in which the said polyhydric alcohol is glycerol.

3. Composition according to claim 1 in which the said short chain aliphatic acid is a fatty acid.

4. Composition according to claim 1 in which the said short chain aliphatic acid is acetic acid.

5. Composition according to claim 1 in which the said short chain aliphatic acid is an hydroxy aliphatic acid.

6. Composition according to claim 1 in which the said short chain aliphatic acid is lactic acid.

7. A textile oil comprising a mineral base oil having a Saybolt Universal viscosity between about 50 and 250 seconds at 100° F. and containing as a scouring assistant an effective amount of a mixed diester of glycerol with a long chain fatty acid of a non-drying fatty oil and a short chain aliphatic acid of less than 4 carbon atoms.

8. Composition according to claim 7 in which said fatty oil is neat's-foot oil.

9. Composition according to claim 7 in which said fatty oil is lard oil.

10. Composition according to claim 7 in which said long chain fatty acid is oleic acid.

11. Composition according to claim 7 in which said long chain fatty acid is obtained from the normally solid fraction of the diglycerides of the fatty acids of a non-drying fatty oil.

12. A textile oil composition comprising a mineral base oil having a Saybolt Universal viscosity between about 50 to 250 seconds at 100° F. and containing as a scouring assistant a mixture of diesters of glycerol, one di-ester being a mixed diester of glycerol with a fatty acid obtained from the normally solid fraction of the diglycerides of the acids of a non-drying fatty oil, and a short chain aliphatic acid of less than 4 carbon atoms, the other diglyceride being a normally liquid diglyceride of the acids of a non-drying fatty oil.

13. Composition according to claim 12 in which said fatty oil is neat's-foot oil.

14. Composition according to claim 12 in which said fatty oil is lard oil.

15. Composition according to claim 1 in which said base oil is a mineral oil having a Saybolt Universal viscosity between about 125° and 175° F., an A. P. I. gravity between about 25 and 32, and a pour point between about 25° and 35° F.

16. Composition according to claim 1 in which the oil is emulsified with water.

17. A textile oil comprising about 94% mineral oil having a viscosity within the approximate range of 50 to 250 seconds Saybolt Universal at 100° F., and about 6% of coconut acetic diester of glycerol.

18. A textile oil comprising about 94% of a mineral base oil having a viscosity within the approximate range of 50 and 250 seconds Saybolt Universal at 100° F., and about 6% of neat's-foot-lactic diester of glycerol.

19. A textile oil comprising about 94% of a mineral base oil having a viscosity within the

approximate range of 50 and 250 seconds Saybolt Universal at 100° F., about 3% of a liquid neat's-foot oil acid diester of glycerol and about 3% of neat's-foot-lactic diester of glycerol.

5 ALFRED C. GOODINGS.

HARRY B. MARSHALL.

HERBERT W. LEMON.